

## UNITED STATES PATENT OFFICE

2,113,418

## PROPELLANT POWDER

Richard G. Woodbridge, Wilmington, Del., assignor to E. I. du Pont de Nemours & Company, Wilmington, Del., a corporation of Delaware

No Drawing. Application October 8, 1936,  
Serial No. 104,667

2 Claims. (Cl. 52—13)

My invention relates to an improved propellant powder of the double-base type, that is, containing both nitroglycerine and nitrocellulose, and to a process for making the same.

Progressive burning nitrocellulose powders of the surface treated type and possessing entirely satisfactory ballistic stability during storage have been known for many years. These powders are made by surface treating powder grains with various moderating agents, preferably those which when liquid are solvents for the nitrocellulose or a portion of the same. Various degrees of improvement in ballistics are obtainable, depending on the ballistic qualities of the powder grains treated, the amount and nature of the moderating agent and the process used for treatment.

Surface treated double-base powders have heretofore been unsatisfactory because of their lack of ballistic stability. This has been attributed to the probability that the moderating agent applied to the surfaces of the powder grains continues to diffuse thruout the grains during storage. This results in objectionable if not also hazardous change in the ballistic properties of the powder and ammunition containing the same.

Brunswig, in his book, *Das Rauchlose Pulver*, page 101, indicates that the surface treatment of powder grains is limited to powder grains having large surface area, and principally to rifle powders, the object being to modify the burning speed on the outer surface and adjacent layers without affecting the interior. He further states that with nitrocellulose powder the effect is caused by supplemental treatment of the surface, while with nitroglycerine powders the same method of treatment cannot be applied and other methods must be used. These other methods discussed by Brunswig do not involve surface treatment of double-base powder grains.

The principal object of my invention is an improved progressive burning double-base powder possessing a high order of ballistic as well as chemical stability. Other objects will appear as the description proceeds.

In accordance with my invention the presence in the double-base powder of any ingredient such as vaseline or starch which might tend to retard the impregnation of the powder grains by the moderating agent and by the process which I use is preferably avoided. Where I find it necessary to obtain flashless results, I prefer to incorporate in the powder a small amount of potassium sulphate in accordance with my U. S. Patent 1,838,345.

The following composition is illustrative of one embodiment of the type of double-base powder grains which I have found satisfactory for subsequent surface treatment by my process:

|                                            | Parts      |
|--------------------------------------------|------------|
| Nitrocellulose of 12.90 to 13.25% nitrogen | 80         |
| Nitroglycerine                             | 20         |
| Potassium sulphate                         | 1          |
| Diphenylamine or other stabilizer          | 0.5 to 1.0 |

The nitrocellulose will preferably be a blend of the type soluble in ether-alcohol with the type insoluble in ether-alcohol, the mixture having a nitrogen content in the neighborhood of 12.90 to 13.25%, but not limited to such. The amount of nitroglycerine may be varied.

The nitrocellulose blend is dehydrated in a press by the conventional method using ethyl alcohol, the excess of alcohol being removed by pressure. The dehydrated nitrocellulose is broken up and placed in the mixing machine, together with the finely pulverized potassium sulphate, if the latter is used. The nitroglycerine, plus stabilizer, is dissolved in acetone and gradually added to the nitrocellulose. The ingredients are mixed for one to two hours, or until a satisfactory colloid of uniform composition is obtained. The colloid is then formed into blocks which are pressed through dies into strings with or without central perforations or into ribbons which are cut up into grains by means of a powder cutting machine. It will be understood that the powder grains referred to subsequently are cylindrical grains with central perforation, although the process described is applicable to grains of other form. The powder grains are dried for several days by means of warm air at a temperature of about 55° C. until the volatile solvents, acetone and alcohol, are substantially removed.

The base grain powder, made as described in the foregoing, may then be surface treated with diethyldiphenylurea in the following illustrative manner:

100 parts by weight of the powder grains are placed in a revolving drum or "sweetie", together with preferably from about two to six parts by weight of diethyldiphenylurea, although these proportions may be varied within the scope of my invention. The powder is then wet and partially covered with water. Steam is admitted to the mixture through an opening in the drum and the water and powder maintained at a temperature of about 75° to 80° C. for one-half hour during which time the drum and contents are

5

10

15

20

25

30

35

40

45

50

55

rotated. As diethyldiphenylurea has a melting point of 71.8° C., the temperature used is sufficient to melt the compound which coats and impregnates the surfaces of the powder grains to some extent because of its solvent action on the nitroglycerine-nitrocellulose composition. The above operation may also be carried out in a jacketed drum heated by steam, hot water or other liquid. Instead of a revolving drum, there may be used any suitable container provided with means of agitation. The ratio of water to powder used will depend to some extent on the apparatus used for surface treating the powder grains. The coated and partially impregnated powder grains are then removed from the drum and subjected to a further impregnation treatment in hot water, preferably at a temperature of about 65° to 75° C., but not limited to such, for about 24 to 72 hours depending on the web thickness of the powder grains in order to cause further impregnating of the nitroglycerine-nitrocellulose colloid by the diethyldiphenylurea.

After the impregnating treatment has been finished, the powder is dried and glazed. The improvement in ballistics which is obtained is very substantial and permanent as will be illustrated by the following ballistic results on two powders of the double-base type, one surface treated according to my invention using diethyldiphenylurea as the moderating agent, and the other powder surface treated with diethylphthalate.

| 35 Pow-<br>der | Surface moderat-<br>ing agent | Inst.<br>vel. at<br>53 ft. | Mean<br>pres-<br>sure        | Storage condition of<br>ammunition                             |
|----------------|-------------------------------|----------------------------|------------------------------|----------------------------------------------------------------|
| 40 A....       | Diethyldiphenyl-<br>urea..... | Feet<br>per<br>second      | Lbs./<br>sq. in.             | Before storage at 55° C.<br>After 30 days storage<br>at 55° C. |
|                |                               | { 3069<br>3022             | { 47,520<br>49,080           | Before storage at 55° C.<br>After 30 days storage at<br>55° C. |
| B....          | Diethylphthalate              | { 2959<br>* 3100           | { 51,290<br>78,800<br>76,850 | Before storage at 55° C.<br>After 30 days storage at<br>55° C. |

45 \*Average of two rounds. All other figures represent average of ten-round series.

Additional tests have confirmed the above results, thus proving that the double-base powder surface moderated in the manner described with diethyldiphenylurea is ballistically stable while powder surface moderated with diethylphthalate was ballistically unstable. 5

My invention is particularly applicable to powder grains intended for use in military rifles and machine guns because it is for this purpose that previous attempts to make progressive burning double base powders of satisfactory ballistic stability have been unsuccessful. It is also to be understood that my process is applicable in general for the preparation of double base powders of the impregnated type for use in all kinds of 10 small arms such as revolvers, pistols, shotguns and rifles. 15

While I prefer to use diethyldiphenylurea as the surface moderating agent, it should be understood that the composition of my double-base powder grains and the process which I use for surface treating the same may tend to facilitate the successful use of other moderating agents having similar properties and performing a like function in a similar manner. 25

As many apparent and widely different embodiments of this invention may be made without departing from the spirit thereof, it is to be understood that I do not limit myself to the foregoing examples or descriptions except as indicated in the following patent claims. 30

I claim:

1. A double-base powder grain having its surface impregnated with diethyldiphenylurea and capable of maintaining its ballistic stability when stored at a temperature of 55° C. for approximately one month. 35

2. A double-base powder grain having its surface treated with diethyldiphenylurea in the presence of water at a temperature of 60 to 75° C., and capable of maintaining its ballistic stability when stored at a temperature of 55° C. for approximately one month. 40

RICHARD G. WOODBRIDGE. 45